

Dec. 9, 1924.

1,518,371

J. TRAQUAIR

METHOD OF COATING PAPER

Filed Dec. 3, 1920



INVENTOR.  
John Traquair,  
BY F. K. Fassett,  
ATTORNEYS.

## UNITED STATES PATENT OFFICE.

JOHN TRAQUAIR, OF CHILlicothe, OHIO, ASSIGNOR TO MEAD PULP AND PAPER COMPANY, OF DAYTON, OHIO, A CORPORATION OF OHIO.

## METHOD OF COATING PAPER.

Application filed December 3, 1920. Serial No. 427,934.

*To all whom it may concern:*

Be it known that I, JOHN TRAQUAIR, a subject of the King of Great Britain, residing at Chillicothe, in the county of Ross and 5 State of Ohio, have invented a new and useful Method of Coating Paper, of which the following is a specification.

My invention relates to the art of applying to paper a coating of pigment to fill up 10 or level the unevenness of the surface and cover the fibers of the paper, and provide a good even printing surface.

In my new method of coating paper I eliminate, among others, two of the most objectionable features which are common to 15 the methods now practiced; namely, the use of excessive quantities of water, and brushing. My method consists briefly, in applying to paper a concentrated suspension in 20 water of finely pulverized mineral or pigment, commonly referred to as "color", drying the paper and then applying a coating of size to bind the color to the paper. When the words "solution" or "color solution" are 25 used they refer to the suspension of pigment in water or other vehicle. That is, of course, not a solution in the strictly chemical sense but in paper coating practice the term "color solution" is commonly used.

30 For the purpose of illustration I have prepared a drawing in which

Fig. 1 shows, diagrammatically, the principal elements of a machine for applying coating to one side of a roll of paper.

35 Fig. 2 shows apparatus for coating paper on both sides simultaneously.

Fig. 3 shows, diagrammatically, the successive stages of the process for coating and sizing paper on one side by my new method.

40 Referring now to Fig. 1, the paper to be coated is taken from the roll 10 and after being coated and dried is rerolled at 11. The paper passes between rolls 12 and 13, the latter of which dips into the solution 45 of color contained in a tub 14. I have obtained the best results from a solution containing approximately one-third water to two-thirds pigment; the preferred consistency is about that of cream. For this purpose I can use any of the substances com-

monly used in coating paper, such as clay, satin white, blanc fixe, etc. It will be seen that at 50 the color accumulates and forms a sort of pool. The zone occupied by this 55 pool has a substantial width, which results

in the paper being exposed to the solution for a more or less definite length of time, according to the diameter of the rolls and the speed of the paper. During this time the paper absorbs a substantial part of the 60 water. Passing between the rolls the pigment is pressed down on the paper, filling the inequalities and forming a fine smooth surface. A sufficient quantity of the water is absorbed by the paper before it passes 65 from between the rolls that the coating is rendered immobile; that is, set or fixed so it can no longer flow. The smooth surface formed by the rolls is therefore retained and thus I eliminate the brushing which has 70 heretofore been an important part of all coating methods.

The coating applied to paper in the above described manner is easily rubbed off, and it is necessary to treat it with a coating of 75 size to fix and bind it to the paper. This may be done in a machine substantially like that shown in Fig. 1, the tub 14 containing size instead of color. But I prefer to pass it through the sizing machine immediately 80 after coating it, thus saving the time of handling it twice. This is shown in Fig. 3, where the paper is coated at A, dried by passing through a drying device B, sized at C, and after being dried again at D is 85 rerolled at E.

If desired the paper may be passed through a second coating and sizing machine, and the other side coated before it 90 is rerolled. All of this will be understood by those skilled in the art and need not be described in greater detail here. In Fig. 2 I show a machine for coating both sides of the paper simultaneously. In this machine the rolls 20 and 21 correspond to rolls 95 12 and 13, respectively, and roll 21 dips into a tub containing color for coating the under side of the paper. For coating the upper surface a roll 22 dips into color contained in a tub 23. The color that is carried up by this roll is removed by a scraper 24 and flowing down the scraper on to roll 20 is deposited by the roll on the upper surface of the paper. After the paper is dried it may be run through a similar machine and both 100 sides sized simultaneously.

Following the custom in paper making machinery I prefer to make one of the rolls of the coating machine soft, preferably rubber covered, and the other hard. The paper 110

may be passed through the machine at a high speed.

The operation of my method is affected by two factors: the absorptivity of the paper and viscosity of the color solution. Paper may be made more or less non-absorptive or water-resisting by the addition of suitable substances to the pulp. For this purpose what is known as rosin size is much used and is put into the beater. According to the 10 quantity of rosin size used paper is known as hard sized or soft sized, the latter absorbing water more readily than the former. In the practice of my method I prefer a 15 paper which would be classed as "soft sized," using a solution of about two parts of pigment to one part of water. Because of the large quantity of water that must be used in the old methods of coating paper, 20 the water resisting quality of hard sized paper has been found advantageous. Soft sized paper becomes mushy and its strength is much impaired by being made very wet. Not only is less water used in coating paper 25 by my method than by others, but as the coating and sizing are done in successive steps, the paper being dried between the steps, the paper is not wetted enough to affect its physical condition materially. In 30 other words, with the older methods a large quantity of water is used in a single step, where in my method a smaller quantity of water is used, and instead of being applied at one time it is used in two parts, that 35 which is put on in the first stage of the operation being evaporated from the paper before the second part is put on. As before stated, the color solution has a consistency about that of cream; obviously, this contains 40 too little water to make the paper soft or otherwise affect its condition materially during the normal operation of my process. The quantity of water applied in the sizing operation is likewise too small to appreciably 45 affect the physical condition of the paper, it requiring only enough water to diffuse the colloidal binding material through the layer of pigment and bind it to the paper. Wetting paper expands it, 50 that is, increases its surface area. One of the advantages of my method is that the expansion of the paper is so slight as to impose no limit on the width of paper which it is practicable to coat thereby. 55 The viscosity of the color solution may be varied to suit the requirements of the paper to be coated. If in using a simple solution of pigment and water the absorption of water is found to be too rapid, it may be 60 slowed down by the addition of a small quantity of a colloidal size. For this purpose one or two per cent of size will usually be sufficient and in any case it will not exceed four or five per cent. The quantity 65 of size used for this purpose is entirely too

small to play any part in binding the coating to the paper, so the second step in the method, that of sizing paper is carried out just the same, whether this small quantity of size is put into the solution or not. If, 70 on the other hand, the absorption is found to be too slow, it may be increased by adding small quantities of suitable chemicals; for example, about one-half per cent of silicate of soda with straight clay color solution, or one per cent gum arabic with lime-containing color solutions, such as satin white. These products have the property of increasing the fluidity or lowering the viscosity of the color solution and thereby 75 accelerating its penetrating quality.

It is seen from the foregoing, that the practice of my new method may begin in the manufacture of the paper to be coated, by making paper having the desired absorptivity. But when this is not done and paper of any given absorptivity is to be coated, the viscosity of the color solution may be varied to suit the paper, in the manner described. I have referred to rosin 90 sized paper, but it is not to be understood that the applicability of my method is limited to rosin sized or any other particular kind of paper. The consistency of the color solution is made such as will enable a coating of desired weight to be deposited on the paper by the roller, and the absorptivity of the paper and viscosity of the solution are so coordinated or adjusted, one to the other, that the coating will be rendered inanimate 95 through absorption of its water by the paper, so that the smooth surface which is imparted to the coating by the rolls will be retained after the paper passes from between the rolls.

There are obvious advantages in reducing the quantity of water used in coating paper: It greatly reduces the cost of drying the paper, for the drying can be done with a far less extensive drying equipment. It 110 also eliminates the common paper coating troubles of grease spots, pin holes and brush marks, and removes the limit on the width of paper that can be coated.

Because of the simplicity of the above described paper coating process, paper may be coated by my method more economically than by any other method of which I am aware. Furthermore, the product is more uniform and combines the advantages of an uncoated paper with those of a coated paper and is superior in quality for certain classes of printing.

Having fully described my new method of coating paper, and described suitable means for carrying out the method, what I claim as my invention, is as follows:

1. The method of coating paper which comprises applying to the paper a layer of "color" comprising a mixture of pigmental 120

matter and water, the quantity of water being limited to that which is required to act as a vehicle for the pigmental matter, and subsequently applying a coating of size whereby to bind the "color" to the paper.

2. The method of coating paper which comprises applying a solution of "color" to the paper, drying the paper and then applying a size to bind the "color" to the paper.

10 3. The method of coating paper which comprises applying a solution of "color" to the paper, then subjecting the paper to pressure between rolls, drying the paper and then applying a coating of size whereby to bind the "color" to the paper.

15 4. The method of coating paper that comprises passing the paper between rolls, one of which is immersed in a solution of "color" and whereby a layer of "color" is deposited on the paper, drying the paper and subsequently applying size to the coated surface, thereby fixing the coating to the paper.

20 5. The method of coating paper that comprises passing the paper between rolls, one of which is immersed in a solution containing approximately two parts of dry "color" to one part of water, both by weight; drying the paper and subsequently applying size to the coated surface whereby to bind the coating to the paper.

25 6. In the coating of paper in which the paper is given a coating of "color" and then a coating of size to bind the coating of "color" to the paper, the method which comprises applying a solution of "color" to the paper and then passing the paper between rolls, the penetrating quality of the solution being adjusted from time to time to the absorptivity of the paper, so that by the time 30 the paper emerges from between the rolls the "color" will have become immobile from loss of its liquid.

35 7. In the coating of paper in which the paper is given a coating of "color" and then a coating of size to bind the coating of "color" to the paper, the method which comprises applying a solution of "color" to the paper and then passing the paper between rolls, the penetrating quality of the solution 40 being adjusted to the absorptivity of the paper, so that by the time the paper emerges from between the rolls the "color" will have.

become immobile from loss of its liquid, drying the paper and then applying a size to bind the "color" to the paper.

55 8. In the coating of paper in which the paper is given a coating of "color" and then a coating of size to bind the coating of "color" to the paper, the method which comprises applying a solution of "color" to the paper and then passing the paper between rolls, the penetrating quality of the solution being adjusted to the absorptivity of the paper by increasing or decreasing the viscosity of the solution, so that by the time 60 the paper emerges from between the rolls the "color" will have become immobile from loss of liquid.

65 9. The method of coating paper, that comprises applying a "color solution" to the paper, said solution having a consistency about that of cream; drying the paper and then applying a solution of colloidal size, said solution containing no more water than is necessary to diffuse the colloidal substance 70 through the coating and bind it to the paper.

75 10. In the coating of paper in which the paper is given a coating of "color" and then a coating of size to bind the coating of "color" to the paper, the method which comprises treating the paper pulp with materials which will give to the paper a predetermined absorptivity; then after the paper is made, applying a solution of "color" and passing the paper between rolls, the solution 80 being made to have viscosity appropriate to the absorptivity of the paper, so that by the time the paper emerges from between the rolls the "color" will have become immobile from loss of its liquid.

85 11. In the coating of paper in which the paper is given a coating of "color" and then a coating of size to bind the coating of "color" to the paper, the method, which comprises applying a layer of "color" comprising a mixture of pigmental matter and water, the quantity of water being limited to that which is required to act as a vehicle for the pigmental matter, and then passing the paper between rolls, whereby the color is 90 pressed down on the paper, filling the inequalities, so as to form a fine smooth surface.

JOHN TRAQUAIR.